

# United States Patent Office

3,330,663

Patented July 11, 1967

1

**3,330,663**  
**SILVER SALTS OF SULFUR-CONTAINING ALIPHATIC CARBOXYLIC ACIDS AS LIGHT-SENSITIVE COMPOUNDS**

Edith Weyde and Anita von König, Leverkusen, Germany, assignors to Agfa-Gevaert Aktiengesellschaft, Leverkusen, Germany, a corporation of Germany  
 No Drawing. Filed July 15, 1965, Ser. No. 472,308  
 Claims priority, application Germany, Aug. 14, 1964, A 46,854

10 Claims. (Cl. 96—94)

This invention relates to a light-sensitive photographic material which contains silver salts of sulfur-containing aliphatic carboxylic acids as light-sensitive compounds. 15 Silver halides are used as light-sensitive compounds in conventional photographic materials. Organic silver salts, for example mercaptides, have also been proposed for this purpose, but have not been used in practice because they are not sufficiently light-sensitive or suffer from 20 other disadvantages.

It is among the subjects of the invention to provide photographic elements, which contain silver salts of sulfur-containing aliphatic carboxylic acids as light-sensitive compounds.

We now have found that silver salts of aliphatic carboxylic acids, the aliphatic chain of which is substituted with a mercapto or organo substituted mercapto group are eminently suitable for photographic purpose. Particular exhibit compounds of the following formula:



2

wherein

$n=1$  or  $2$ ,

$R=$ alkyl, preferably with up to 18 carbon atoms, aralkyl such as benzyl or phenylethyl, aryl such as phenyl or naphthyl, or heterocyclic rings such as diazolyl, oxazolyl, triazolyl, oxidiazolyl, thiadiazolyl, azaindenyl, preferably tetra- or pentaazaindenyl, benzthiazolyl, naphthiothiazolyl, benzoaxazolyl, naphthoxazolyl, pyridyl, quinolinyl, pyrimidyl, quinoxalinyl, quinazolinyl, which radicals may in turn be substituted, for example, by alkyl, preferably with up to 18 carbon atoms, aryl such as phenyl or naphthyl, hydroxyl, alkoxy with preferably up to 12 carbon atoms, aroxy such as phenoxy, acyl preferably acyl derived from aliphatic carboxylic acids having up to 18 carbon atoms, amino, alkylamino, the alkyl groups of which having up to 5 carbon atoms, acylamino with preferably acyl groups being derived from aliphatic carboxylic acids having up to 18 carbon atoms or aryl-substituted amino preferably a phenylamino, mercapto groups, mercapto groups substituted with alkyl having up to 18 carbon atoms, a phenyl, a naphthyl or a heterocyclic radical, halogen such as chlorine or bromine, sulfo groups or carboxyl groups and the like, and

25  $X=$ a branched or unbranched alkylene chain having preferably up to 12 carbon atoms in particular 1-5 carbon atoms, whereby the alkylene chain can further be substituted with aryl preferably a phenyl, hydroxyl, alkoxy, halogen such as chlorine or bromine and the like. Sulfur-containing aliphatic carboxylic acids useful according to the invention, include the following:

184° C.

Beilstein, vol. 3,  
 page 249.

44° C.

Beilstein, vol. 3,  
 3rd Supp. vol.  
 part 1, page 416.

Beilstein, vol. 3,  
 3rd Supp. vol.  
 part 1, page 417.

Beilstein, vol. 3,  
 3rd Supp. vol.  
 part 1, page 417.

Beilstein, vol. 3,  
 3rd Supp. vol.  
 part 1, page 418.

Beilstein, vol. 3,  
 page 250.

J. Am. Soc. 74, 130° C  
 page 5577 (1952).

56-59° C.

Beilstein, vol. 3,  
 3rd Supp. vol.  
 part 1, page 413.

56° C.

Beilstein, vol. 3,  
 page 253.

14.   
CH<sub>3</sub>—CH<sub>2</sub>—S—CH<sub>2</sub>—COOH
15.   
CH<sub>3</sub>  
S—CH—COOH  
CH<sub>2</sub>  
S—CH—COOH  
CH<sub>3</sub>
16.   
CH<sub>3</sub>  
S—CH—COOH  
(CH<sub>2</sub>)<sub>2</sub>  
S—CH—COOH  
CH<sub>3</sub>
17.   
HOOC—CH—CH<sub>2</sub>—S—CH<sub>2</sub>—COOH  
NH<sub>2</sub>

Beilstein, vol. 3,  
page 291.

18.   
COOH  
CH<sub>2</sub>  
CH—S—CH<sub>2</sub>—COOH  
COOH
19.   
COOH  
CH<sub>2</sub>  
CH—S—C<sub>12</sub>H<sub>25</sub>  
COOH

J. Am. Chem. Soc.  
vol. 66, page  
1758 (1944).Beilstein, vol. 3,  
3rd Supp. vol.  
part 2, page 924.

- 20.

101° C.

21.   
COOH      COOH  
CH<sub>2</sub>      CH<sub>2</sub>  
OH—S—S—CH  
COOH      COOH

Beilstein, vol. 3,  
page 439.

22.   
CH<sub>2</sub>—COOH  
S  
CH<sub>2</sub>—CO—NH—C<sub>6</sub>H<sub>5</sub>

Beilstein, vol. 12,    103-104° C.  
page 485.

23.   
CH<sub>2</sub>—COOH  
S  
CH<sub>2</sub>—CO—NH—C<sub>6</sub>H<sub>5</sub>  
CH<sub>3</sub>

114° C.

- 24.

Beilstein, vol. 13,  
1st Supp. vol.,  
page 175.

122-123° C.

- 25.

214° C.

- 26.

102° C.

- 27.

5



6

144° C.

Beilstein, vol. 6,  
page 313.

124° C.



198° C.

Beilstein, vol. 6,  
page 463.

60-61° C.

Beilstein, vol. 6,  
page 463.Beilstein, vol. 6,  
page 328.Beilstein, vol. 6,  
2nd Supp. vol.,  
page 343.Beilstein, vol. 6,  
1st Supp. vol.,  
page 150.U.S. Patent  
2,897,081.Beilstein, vol. 6,  
1st Supp. vol.,  
page 195.Beilstein, vol. 6,  
page 337.241° C. (decom-  
position)

7



8

175° C. (decomposition)

200° C.

Ann. 353, page 127  
(1907).

126° C.

J. Am. Soc. 74,  
page 5577 (1952).Beilstein, vol. 10,  
2nd Supp. vol.,  
page 73.Beilstein, vol. 10,  
2nd Supp. vol.,  
page 137.Beilstein, vol. 10,  
page 950.Beilstein, vol. 6,  
page 623.

161° C.

Beilstein, vol. 22,  
2nd Supp. vol.,  
page 167.Beilstein, vol. 22,  
2nd Supp. vol.,  
page 302.Beilstein, vol. 22,  
2nd Supp. vol.,  
page 164.

9



10

120-120.5° C.



91° C.

Beilstein, vol. 23,  
1st Supp. vol.,  
page 119.Beilstein, vol. 25,  
page 62.

193° C.

Beilstein, vol. 25,  
page 15.

187° C.

270° C. (decom-  
position)

169° C.

230-340° (decom-  
position)

196° C.

Beilstein, vol. 26,  
page 128.211° C. (decom-  
position)



269° C. (decomposition)

205° C. (decomposition)

170° C. (decomposition)

239° C.

U.S. Patent  
2,819,965.

302° C. (decomposition)

Bellstein, vol. 27,  
page 244.

180-182° C. (decomposition)

U.S. Patent  
2,819,965.

270° C. (decomposition)

196° C.

Beilstein, vol. 23,  
2nd Supp. vol.,  
page 321.

13



14

296° C. (decomposition)



300° C. (decomposition)

Beilstein, vol. 26,  
1st Supp. vol.,  
page 82.

165° C.



156° C.

Beilstein, vol. 26,  
1st Supp. vol.,  
page 169.Beilstein, vol. 27,  
2nd Supp. vol.,  
page 787.Beilstein, vol. 27,  
1st Supp. vol.,  
page 612.

159° C.



150° C.



Uncrystallized



61° C.



42° C.



150° C.



45° C.

15



16

64° C.

84° C.

205° C.

194° C.

195° C.

196° C.

260° C. (decomposition)

192° C.

158° C.

104° C.

128° C.

178° C.

117° C.

Beilstein, vol. 3, 101° C.  
page 312.Beilstein, vol. 6, 58-60° C.  
2nd Supp. vol.,  
page 293.Beilstein, vol. 6, 87-89° C.  
2nd Supp. vol.,  
page 293.



105° C.

114-115° C.

122-123° C.

135-136° C.

Uncrystallized



129-130° C.

Beilstein, vol. 6,  
2nd Supp. vol.,  
page 306.

133° C.

Beilstein, vol. 6,  
2nd Supp. vol.,  
page 313.

41-43° C.



50-53° C.





109° C.

146° C.

181-182° C.

95° C.

202° C.

J. Am. Soc. 74,  
page 3886, (1952). 96° C.

128° C.

123° C.

184° C.

190° C.

126° C.

105° C.

Preferred are compounds of the above general formula wherein X is a methylene group which can be substituted as described hereinbefore. Particularly suitable are thioaliphatic carboxylic acids wherein R is an alkyl more particularly a phenyl-substituted aminoalkyl of the formula



wherein the benzene rings can be substituted as disclosed hereinbefore.

70 The compounds may be prepared by the processes described in the publications referred to in the table. The remaining compounds may be prepared from the corresponding mercaptans and organic halogen compounds or halogen carboxylic acids in alkaline solution by processes similar to those described in Houben-Weyl, vol. 9, pages

103 to 113. The compounds can be isolated in the form of free acids or as alkali metal salts. The compounds can be purified by recrystallisation from or by solution and reprecipitation from water or alcohol. This is more fully described in the following examples:

PREPARATION OF S-[2-n-OCTYLTHIO-1,3,4-THIADIAZOLYL-(5)]-THIOGLYCOLIC ACID—COMPOUND 96

26.5 g. ( $\frac{1}{10}$  mol) of 2-n-octylmercapto-5-mercaptop-thiadiazole-(1,3,4) are dissolved in 100 ml. of 1 n-sodium hydroxide solution and, after the addition of 10.5 g. of monochloroacetic acid, the solution is heated for 15 minutes on a steam bath while stirring. After cooling to 60° C., 9.4 g. of soda are added in portions, after the solution is heated for 2 hours on a steam bath. The product is precipitated by acidification with dilute acetic, and is purified by recrystallisation from methanol. Yield: 20 g., M.P. 63° C.

PREPARATION OF THE SODIUM SALT OF S-[2-n-BUTYLTHIO-1,3,4-THIAZOLYL-(5)]-THIOGLYCOLIC ACID—COMPOUND 98

103 g. ( $\frac{1}{2}$  mol) of 2-n-butylmercapto-5-mercaptop-thiadiazole-(1,3,4) are dissolved in 800 ml. of a 2.5% by weight sodium hydroxide solution and, after the addition of 63 g. of monochloroacetic acid, the solution is heated for 15 minutes on a steam bath while stirring. 50 g. of soda are then added in portions at about 60° C., after which the solution is heated for 3 hours on a steam bath and after cooling the product is precipitated by acidification with 50% aqueous acetic acid. The crude product is purified by washing with water. The resulting 65 g. of crude product are dissolved in an equivalent quantity of 5% aqueous soda solution, after which the sodium salt of the product is isolated in the form of fine needles by concentration. The salt melts at 218° C. after washing with acetone and drying in vacuo.

Compounds 129-135 are prepared by reacting a Schiff base with a mercapto-substituted aliphatic carboxylic acid as described for example by Stacy et al., J.A.C.S. 77, 3869, 1955.

The preparation of conventional silver halide emulsion involves three separate steps: (1) precipitation of the silver halide in the presence of a protective colloid preferably gelatin and physical or Ostwald ripening, (2) flocculation and freeing of the emulsion of excess water-soluble salts, and (3) the chemical or after-ripening to obtain increased speed and sensitivity (compare Mees "The Theory of the Photographic Process").

The novel photographic emulsions of the present invention can be prepared in analogous manner.

The silver salts are prepared from equimolar quantities of the thioaliphatic carboxylic acid and the soluble salt such as silver nitrate. The reaction takes place in an aqueous solution of the reaction components, preferably in the presence of a protective colloid such as gelatin, polyvinyl alcohol, or sodium alginate. Depending on the type of thioaliphatic carboxylic acid used, the components are reacted in a molar ratio about 1:1. That molar ratio relates to the number of carboxyl groups. Thus an acid which contains two carboxyl groups is preferably reacted with 2 mols of water-soluble silver salt such as silver nitrate. Acids which contain 3 or more carboxyl groups are preferably reacted with a least 2 mols of silver salt. The most effective and suitable molar ratio will be apparent to those skilled in the art upon making the ordinary tests and observations customarily used in the art of emulsion making. It has been found that an excess of water soluble silver salt produces fogging in the photographic emulsion. On the other hand, an excess of thioaliphatic carboxylic acid up to about 10 mol percent reduce the fog level without affecting sensitivity. A higher excess of the thioaliphatic carboxylic acid is not desirable since the light-sensitivity of the silver salts of the said acid is considerably reduced.

Precipitation of the silver salt in the presence of a film-forming binding agent produces an emulsion suitable for coating.

Water soluble organic and inorganic silver salts as well as silver complexes may be used for the reaction with the thioaliphatic carboxylic acid. The anion of the silver salts used to prepare the silver salts according to the invention may itself be used in the photographic emulsion, for example, as a hardening agent for adjusting the required pH-value.

The silver salts according to the invention may also be employed in admixture with one another or with conventional silver halides.

The type of water-permeable binding agents which can be used include those which are known to be satisfactory for dispersing silver halides. These colloids comprise preferably gelatin which however can be wholly or partially replaced by other film-forming natural or synthetic materials such as proteins for instance albumin or casein, alginic acids or derivatives thereof by alkali salts of alginic acid, esters of alginic acids in particular esters with lower aliphatic alcohols preferably glycols such as propylene glycol, carboxylalkylcellulose such as carboxymethylcellulose, alkylcellulose, such as methylcellulose or hydroxyethylcellulose, starch, starch ethers or esters such as ester with lower aliphatic alcohols having up to 5 carbon atoms or alkyl ethers the ether group of which has up to 5 carbon atoms, caragenates, polyvinylalcohol, partially saponified polyvinylacetate, polyvinyl pyrrolidone and the like.

The emulsion of the invention contains between 1 and 80 preferably 2 and 25 g. of silver in the form of the inventive silver salt per litre of emulsion. The final light-sensitive layers contain between 0.05 and 10 preferably between 0.2 and 2 g. silver in the form of the inventive silver salt per square meter. The thickness of the layers is between 0.5 and 30 microns, preferably 6-15 $\mu$ . The emulsion of the present invention can be chemically sensitized by any of the accepted procedures. The emulsions can be treated with salts of the noble metals such as ruthenium, rhodium, palladium, iridium and platinum.

Suitable compounds are well known in the art. The emulsions can also be sensitized with gold salts as described by R. Koslowsky, Z. wiss. photo. 46, 65-72 (1951).

The emulsion can also be chemically sensitized with reducing agents such as stannous salts, polyamines, sulfur compounds, such described in the U.S. Patent No. 1,574,944, polyethylene oxides and the like.

The emulsion can also be optically sensitized with the ordinary sensitizing dyes, cyanines or merocyanines. The emulsions of the present inventions and the light-sensitive emulsion layers have a pH of between 1 and 6, preferably between 2.5 and 5. The emulsions can be stabilized with any of the known stabilizers such as mercury compounds, triazoles, azaindenes, such as disclosed by Birr in Z. wiss. phot., vol. 47 (1952) 2-28.

The emulsions may be hardened by any suitable hardener, such as formaldehyde, halogen substituted aliphatic acids such as mucobromic acid.

Example 1  
30 ml. of a 40% aqueous citric acid solution and 20 g. of diethyldisulfide-1,2,1',2'-tetracarboxylic acid (compound 21) dissolved in an equimolar quantity of aqueous sodium hydroxide solution, are added to 1 litre of an 8% aqueous gelatin solution at 40° C. 100 ml. of a 10% aqueous solution of silver nitrate are then added with vigorous stirring and digested for a few minutes at 40° C. After the addition of a wetting agent, for example 5 ml. of a 30% by weight aqueous saponin solution, and of a hardening agent, for example 1 ml. of a 30% by weight formaldehyde solution, the emulsion is coated in known manner on to a paper sheet or on to transparent support of celluloseacetate and dried. The sensitivity of the coated material is similar to that of conventional photographic silver chloride contact-copying paper, After exposure,

the material may be developed, fixed and treated with water in the usual way. The following developer mixture is used:

|                                                  | G. |
|--------------------------------------------------|----|
| p-Methylaminophenol                              | 1  |
| Anhydrous sodium sulfite                         | 13 |
| Hydroquinone                                     | 3  |
| Anhydrous soda                                   | 26 |
| and                                              |    |
| Potassium bromide, dissolved in 1 litre of water | 1  |

Since the silver salt precipitates in a very fine-grained form, these emulsions may be prepared with a comparably low silver content without reducing the density of the resulting images. Instead of diethyldisulfide-1,2,1',2'-tetracarboxylic acid, it is also possible to employ the following compounds in the quantities indicated:

20 g. of s-[6-methylpyrimidyl-(2,4)]-bis-thioglycollic acid (compound 63) 22 g. of s-[7-sulfo-naphtho-2',3':4,5-oxazolyl-(2)]-thioglycollic acid (compound 82) 21 g. of s-[7-sulfo-5-chloro-benzoxazolyl-(2)]-thioglycollic acid (compound 74) 27 g. of s-[2-n-dodecylthio-1,3,4-thiadiazolyl-(5)]-thioglycollic acid (compound 98) 17 g. of s-[2-anilino-1,3,4-thiadiazolyl-(5)]-thioglycollic acid (compound 103).

#### Example 2

30 ml. of a 40% aqueous solution of citric acid are added to 1 litre of an 8% aqueous gelatin solution, and the solution is heated to 45° C. 20 g. of carboxymethyl-mercaptosuccinic acid (compound 18) dissolved in an equimolar quantity of aqueous sodium hydroxide solution are added, after which precipitation is carried out while stirring vigorously with 100 ml. of a 10% aqueous silver nitrate solution. Before coating, 3 ml. of a 1% alcoholic solution of 1-phenyl-5-mercaptotetrazole, 5 ml. of a 1% alcoholic solution of benzotriazole, 1 ml. of a 30% aqueous formaldehyde solution and 5 ml. of 30% aqueous solution of saponin are added. The emulsion is applied in known manner on to a sheet of paper and is then dried.

Since the silver salt dissolves readily in an alkaline sulfite solution, this material may be employed as light-sensitive photographic material in the silver salt diffusion process without applying a silver salt solvent such as sodium thiosulfate.

The exposed element is developed in the usual way using thiosulfate-free transfer materials, containing development nuclei and thiosulfate-free aqueous developers. The materials are processed in accordance with common practice. After the materials have been separated, an excellent copy of the original is obtained in the transfer material.

#### Example 3

2 ml. of a 40% aqueous solution of citric acid are added to 1 litre of an 8% aqueous gelatin solution, and the solution is heated to 40° C. 22 g. of s-[2-n-octylthio-1,3,4-thiadiazolyl-(5)]-thioglycollic acid (compound 96), dissolved in an equimolar quantity of an aqueous sodium hydroxide solution, are then added, after which precipitation is carried out while stirring vigorously with 100 ml. of a 10% aqueous solution of silver nitrate. Before coating, 125 g. of crystalline sodium acetate, 5 g. of potassium metabisulfite, 5 g. of sodium 4-diethylaminobenzene-aminomethane sulfonate-(1) and 5 ml. of a 30% aqueous solution of saponin, are added. The emulsion is cast in known manner on to a sheet of paper and dried. After exposure, the material may be developed under heat or used as light-sensitive material for a developer sublimation process, for example as described in German patent specification No. 1,159,758.

#### Example 4

30 ml. of a 40% aqueous solution of citric acid and 18 g. of compound 126 dissolved in water which, if desired,

can be mixed with a small amount of aqueous sodium hydroxide solution to facilitate solution, are added at 40° C. to 1 litre of an 8% by weight aqueous gelatin solution. 100 ml. of a 10% aqueous solution of silver nitrate are then added with vigorous stirring and digested for a few minutes at 40° C. After the addition of a wetting agent, for example 5 ml. of 30% by weight aqueous solution of saponin, and a hardening agent, for example 1 ml. of a 30% by weight formaldehyde solution, the emulsion is applied in known manner into a sheet of paper or into a transparent support for example of polyethylene terephthalate and dried. The sensitivity of the coated material is similar to that of conventional photographic silver chloride contact-copying papers. After exposure, the material may be developed, fixed and treated with water in the usual way. For example the developer composition referred to in Example 1 can be used. Since the silver salt is precipitated in a very fine-grain form, these emulsions can be prepared which have a low silver content as compared with a conventional silver halide emulsion without affecting the density of the final images. Instead of compound 126, it is also possible to employ the following compounds in the quantities indicated: 14 g. of compound 111; 13 g. of compound 121; 21 g. of compound 125; 16 g. of compound 124 or 16 g. of compound 119.

#### Example 5

30 ml. of a 40% aqueous solution of citric acid are added to 1 litre of an 8% by weight aqueous gelatin solution, and the solution is heated to 45° C. 15 g. of compound 109 dissolved in water mixed with a little aqueous sodium hydroxide solution are then added, after which precipitation is carried out while stirring vigorously with 100 ml. of a 10% by weight aqueous solution of silver nitrate. Before casting, 3 ml. of a 1% by weight alcoholic solution of 1-phenyl-5-mercaptotetrazole, 5 ml. of a 1% by weight alcoholic solution of benzotriazole, 1 ml. of a 30% by weight formaldehyde solution and 5 ml. of a 30% aqueous solution of saponin are added. The emulsion is applied to a sheet of paper in known manner and dried.

The material is exposed and further processed in accordance with the silver salt diffusion process by developing the exposed light-sensitive layer, while in contact with a transfer sheet containing development nuclei and separating the sheets when the transfer of the silver salt is completed. Since the silver salt dissolves readily in an alkaline sulfite solution, it is not necessary to apply a silver salt solvent such as sodium thiosulfate in the developer bath or in the transfer sheet. An excellent copy of the original is obtained.

#### Example 6

2 ml. of a 40% aqueous solution of citric acid are added to 1 litre of an 8% by weight aqueous gelatin solution, and the solution is heated to 40° C. 15 g. of compound 118 dissolved in water mixed with a small amount of sodium hydroxide solution are then added, after which precipitation is completed while stirring vigorously with 100 ml. of a 10% by weight aqueous silver nitrate solution. Before casting, 125 g. of crystalline sodium acetate, 5 g. of potassium metabisulfite, 5 g. of sodium 4-diethylaminobenzene-1-aminomethane sulfonate and 5 ml. of a 30% aqueous solution of saponin, are added. The solution is applied to a sheet of paper and dried.

After exposure, the material can be developed under heat, or used as a light-sensitive material for a developer sublimation process as described for example in German patent specification No. 1,159,758.

We claim:

1. A light-sensitive photographic element having at least one light-sensitive silver salt emulsion layer in which the essential light-sensitive silver salt is a silver salt of an aliphatic carboxylic acid the aliphatic chain of which is substituted with an organo substituted mercapto group.

2. A light-sensitive photographic element as defined in claim 1, wherein the light-sensitive silver salt is a salt having the following formula



wherein

R represents a member of the group consisting of alkyl having up to 18 carbon atoms, aralkyl, a radical of the benzene series, a radical of the naphthalene series and a heterocyclic ring; and

X represents an alkylene radical having up to 5 carbon atoms.

3. A light-sensitive photographic element as defined in claim 1, wherein the water-permeable binding agent of the light-sensitive layer consists essentially of at least one member of the group consisting of gelatine, albumin, alginic acid, alkali salts of alginic acid, esters of alginic acid, alginic acid amide, polyvinylalcohol, partially hydrolyzed polyvinylacetate, polyvinylpyrrolidone, starch, carboxyalkylcellulose and alkycellulose.

4. A light-sensitive photographic element as defined in claim 1, wherein the light-sensitive silver salt emulsion layer has a pH between 1 and 6.

5. A light-sensitive photographic element as defined in claim 2, wherein X is a methylene group.

6. A light-sensitive photographic element as defined in

20

5 claim 2, wherein the light-sensitive silver salt is a salt of an alkylene-bis-thioglycollic acid.

7. A light-sensitive photographic element as defined in claim 2, wherein the light-sensitive silver salt is a salt of an S-carboxyalkyl-thioglycollic acid.

8. A light-sensitive photographic element as defined in claim 2, wherein R is a heterocyclic radical of the group consisting of a quinolyl, a pyrimidyl, a quinoxalyl, quinazolyl, phthalazyl, triazolyl and thiazolyl.

9. A light-sensitive photographic element as defined in claim 2, wherein R is a methyl group which is substituted with a phenyl group and a phenylamino group.

10. A light-sensitive photographic element as defined in claim 1, and in which the light-sensitive silver salt is a silver salt of:



No references cited.

25 NORMAN G. TORCHIN, *Primary Examiner.*

C. E. DAVIS, *Assistant Examiner.*

UNITED STATES PATENT OFFICE  
CERTIFICATE OF CORRECTION

Patent No. 3,330,663

July 11, 1967

Edith Weyde et al.

It is hereby certified that error appears in the above numbered patent requiring correction and that the said Letters Patent should read as corrected below.

Column 11, for the lower portion of formula 77 reading "N" read -- S --; column 13, for the left-hand portion of formula 92 reading "H<sub>2</sub>C<sub>3</sub>" read -- H<sub>7</sub>C<sub>3</sub> --; column 19, for the lower portion of formula 132 reading "--N" read -- --NH --; column 20, line 70 for "processess" read -- processes --; column 21, line 20, for "THIAZOLYL" read -- THIADIAZOLYL --; column 22, line 23, for "carboxylalkylcellulose" read -- carboxyalkylcellulose --; column 23, line 10, for "dissolved" read -- dissolved --; column 25, line 20, for "alkycellulose" read -- alkylcellulose --.

Signed and sealed this 17th day of September 1968.

(SEAL)

Attest:

Edward M. Fletcher, Jr.

Attesting Officer

EDWARD J. BRENNER

Commissioner of Patents